

## UNITED STATES PATENT OFFICE

2,006,598

CORROSION-RESISTANT AND MALLEABLE  
ALLOY

Wolf Johannes Müller and Moritz Niessner,  
Vienna, Austria, assignors to Oesterreichische  
Dynamit Nobel Aktiengesellschaft, Vienna,  
Austria, a firm of Austria

No Drawing. Application June 30, 1933, Serial  
No. 678,472. In Austria July 8, 1932

## 5 Claims. (Cl. 75—1)

This invention relates to corrosion-resistant and malleable alloys.

5 Gamma brass, that is to say, copper-zinc-alloys containing from 31 to 40% of copper, are known in the literature. Such alloys are distinguished by a low copper content, and are more corrosion-resistant than the generally used brass alloys of high copper content of the alpha and alpha+beta fields, and containing for example, 10 68 to 72% of copper. It is however, impossible to employ the gamma alloys, poor in copper, industrially, since these alloys are extraordinarily hard and brittle, and can therefore not be worked.

The surprising observation has now been made 15 in accordance with the present invention, that by the addition of a few per cent of a metal soluble in gamma brass, such as nickel or more advantageously cobalt—the amount of the added metal lying within the solubility limits in gamma brass—and advantageously by the simultaneous addition of nickel and cobalt, alloys are obtained 20 which exhibit the excellent anti-corrosion properties of the gamma alloys, but which are admirably adapted to be mechanically worked.

25 Alloys are particularly useful which contain said additional metal in amounts below 10%, that is to say, for example, alloys containing less than 10% of cobalt or less than 10% of cobalt and nickel jointly. The simultaneous employment of 30 cobalt and nickel enables the same effects to be obtained with a substantially smaller cobalt content than when using cobalt alone.

The alloys of the present invention are also distinguished by a high resistance to erosion.

35 The following are examples of compositions of alloys in accordance with the invention, the parts being given by weight:—

- |                            |    |
|----------------------------|----|
| (1) 38 to 33% of copper    | 5  |
| 3 to 8% of cobalt          |    |
| Remainder zinc.            |    |
| (2) 38 to 32% of copper    | 10 |
| 4 to 9% of nickel          |    |
| Remainder zinc.            |    |
| (3) 38 to 33% of copper    | 15 |
| 1 to 6% of cobalt          |    |
| Approximately 4% of nickel |    |
| Remainder zinc.            |    |

What we claim is:

1. Corrosion-resistant, mechanically workable alloys which consist substantially of a copper-zinc alloy containing copper in an amount corresponding to gamma-brass and an addition of 15 from 3 to 10 percent of one of the elements cobalt and nickel.

2. Corrosion-resistant, mechanically workable alloys according to claim 1, containing at least 20 5 to 6 percent of cobalt.

3. Corrosion-resistant, mechanically workable alloys according to claim 1, containing at least 7 to 8 percent of nickel.

4. Corrosion-resistant, mechanically workable 25 alloy having the following composition:

|        |           |
|--------|-----------|
| Copper | 33 to 38% |
| Cobalt | 3 to 8%   |
| Zinc   | Remainder |

5. Corrosion-resistant, mechanically workable 30 alloy having the following composition:

|        |           |
|--------|-----------|
| Copper | 32 to 38% |
| Nickel | 4 to 9%   |
| Zinc   | Remainder |

WOLF JOHANNES MÜLLER.  
MORITZ NIESSNER.